

# UNITED STATES PATENT OFFICE.

ENRIQUE A. TOUCEDA, OF ALBANY, NEW YORK.

## ALLOY FOR BEARING METALS.

No. 897,431.

Specification of Letters Patent.

Patented Sept. 1, 1908.

Application filed November 27, 1907. Serial No. 404,150.

*To all whom it may concern:*

Be it known that I, ENRIQUE A. TOUCEDA, a citizen of the United States, residing at Albany, in the county of Albany and State of New York, have invented certain new and useful Improvements in Alloys for Bearing Metals; and I do hereby declare the following to be a full, clear, and exact description of the invention, such as will enable others skilled in the art to which it appertains to make and use the same.

This invention relates to certain new and useful improvements in alloys for white bearing metals.

It is well known by those familiar with the composition and uses of a bearing metal that it should possess—

First. Softness, that is, ability to adapt itself to the irregularities of the journal-surfaces with which it is in contact, and consequently to run at a low temperature.

Second. As fine a grain as possible coincident with the greatest possible toughness and hardness. This means high pressure capacity, resistance to shock and vibration, low co-efficient of friction, and durability.

Third. Fusibility and fluidity in order that sharp and homogeneous castings may be produced, and

Fourth. Cheapness.

It has been stated by one of the highest authorities engaged in the manufacture of white bearing metals that "the ideal bearing metal will be attained when it combines in the greatest degree the soft yielding properties of lead, with the toughness and hardness of copper etc." It is recognized by all of those qualified to express an opinion upon the subject that if lead could be made to remain in place it would be superior as a bearing metal to any other metal or combination of metals known.

In the manufacture of white bearing metals as at present practiced it is usual to employ lead and to harden the same by the addition of antimony. While the addition of antimony hardens the lead, it not only makes the grain coarser, but each per cent. of addition rapidly decreases its ductility until a condition is reached where the alloy is extremely brittle. This result and condition is well known to those skilled in the art and hence many endeavors have been made to discover a substitute which should be free from this effect. With this end in view it has been suggested to add both antimony

and copper to the lead with the dual object of hardening and toughening the lead, but where high speed and pressure, or high speed combined with shock and vibration are met with, it has been found that such an alloy will have but a short life. For this class of service therefore, it has been found necessary to substitute for the lead in whole or in part, tin, which with the antimony and the copper produces a finer grained and tougher alloy though at considerably increased cost owing to the fact of tin being worth many times the value of lead.

It may be confidently asserted that more than 99% of all white bearing metals now manufactured and in use are composed of some combination of the four metals hereinbefore named, and of these four antimony is the one essential constituent.

My invention has for its object the production of a white bearing metal which shall possess all of the recognized good antifriction properties of lead, with the additional properties of hardness and toughness, and with this end in view my invention consists of an alloy composed of lead and cadmium.

Many experiments in service and laboratory tests demonstrate the facts that no practical benefit is obtained from the cadmium addition, when hardening and toughening are considered, if the cadmium addition be less than 2.75% of the lead or other metals that may be used in the alloy. When the alloy is made up with this percentage of cadmium it is suitable only for the low pressure low speed work, free from shock, but it outwears more costly bearings that are considered suitable for the same purpose. For higher speeds and greater loads, the cadmium addition must be increased for the reason that the alloy must be made harder to withstand the increased load and speed. The cadmium addition for these cases should be in the neighborhood of 8%. For these same speeds and loads, but when the bearing may at the same time be subjected to shock, the cadmium must be increased to 11%. For the pinion end of armatures of electric cars, where the cars are light and average speed maintained, due to shock and hard service the cadmium must be increased to 14% and on heavier cars to 18%. For extremely heavy service where the load, speed and shock are very severe, the cadmium addition must preponderate over the lead or lead and other metals.

In intelligently designing bearings embodying my invention the load, speed, and other conditions must be considered as is well understood by those skilled in the art, 5 but from the data herein given those skilled in the art will readily be able to make a suitable bearing for any purpose.

I do not deem it necessary to give directions for the melting of the metals for the 10 reason that those skilled in the art are familiar with the requirements and the literature on the subject is old and well known.

Having given the percentages of cadmium necessary under the conditions recited for 15 securing the desired hardness and toughness of the alloy, I shall hereinafter refer to the percentage to be employed as sufficient to produce the desired result.

I have found from practical experience 20 that even in those instances where the service is extremely drastic and severe, and where only those babbitts in which the base was all tin would stand for any length of time, and where babbitts with an all lead 25 base could not be used owing to rapid failure, that bearings composed of lead hardened and toughened with cadmium have power to be quite as much superior to an all tin base, as the latter is to the all lead base, when these 30 two metals were hardened and toughened with copper and antimony. I have found further, that an alloy such as I have produced in which lead is used in whole or in part as the base, that such base is made 35 harder, stiffer and tougher by the addition of cadmium and is therefore capable of sustaining more weight per square inch of bearing.

In the manufacture of my improved alloy a percentage of cadmium sufficient to harden 40 and toughen the lead is employed, the hardness increasing with the percentage of cadmium added. For instance the percentage of cadmium should be adjusted for the character of service desired of the bearing, and I 45 therefore wish it to be understood that my invention resides broadly in an alloy com-

posed of lead and a percentage of cadmium sufficient to harden and toughen the lead to such degree as may be desired according to the service to be performed.

While lead alone with a percentage of cadmium sufficient to toughen and harden the lead as hereinbefore explained produces an alloy adapted for use wherever a white bearing metal is required, I desire it to be especially understood that I do not confine myself to the use of the two bodies named, but that I may apply the cadmium to any combination of metals heretofore used to produce alloys for white bearing metals, or to any 55 combination of metals which may herein-after be employed, the spirit of my invention residing broadly in the incorporation of cadmium in any such alloys, in such percentage as will produce the hardening and toughening 60 effect upon the lead constituent.

Having described my invention so that those skilled in the art may know how to produce the improved alloy and appreciate all of its advantages, what I claim as new and desire to secure by Letters Patent is—

1. A bearing composed of an alloy of lead and cadmium.
2. A bearing composed of an alloy composed of lead and cadmium, in which the 75 lead predominates.
3. A bearing composed of an alloy one of whose ingredients is lead, toughened and hardened by the presence of cadmium.
4. A bearing composed of an alloy of lead 80 and other metals, said alloy being hardened and toughened by the presence of cadmium.
5. A bearing metal composed of an alloy whose base is lead, hardened and toughened by the presence of cadmium.

In testimony whereof, I have signed my name to this specification in the presence of two subscribing witnesses.

ENRIQUE A. TOUCEDA.

Witnesses:

D. G. STUART,  
JNO. J. HAROWER.